

## UNITED STATES PATENT OFFICE

1,952,049

## ALUMINUM-BERYLLIUM ALLOY

Robert S. Archer, Milwaukee, Wis., and William L. Fink, Oakmont, Pa., assignors to Aluminum Company of America, Pittsburgh, Pa., a corporation of Pennsylvania

No Drawing. Application June 17, 1932  
Serial No. 617,863

2 Claims. (Cl. 75—1)

This application is a continuation in part of our copending application Serial No. 462,403, filed June 19, 1930, which, in turn, is a continuation in part of our copending application Serial No. 327,176, filed December 19, 1928, and on which Patent No. 1,774,542 was issued September 2, 1930, which, in turn, is a division of our patent application Serial No. 150,141, filed November 22, 1926, on which Patent No. 1,716,943 was issued June 11, 1929. The claims of this application are directed toward the disclosure in said last mentioned patent application, of aluminum base alloys containing beryllium and magnesium.

15 The invention relates to aluminum base alloys containing beryllium, the object being to provide an improved aluminum-beryllium alloy which has substantial advantages without as well as with heat treatment.

20 Because of its low density, beryllium is a desirable alloying element for many purposes for which light aluminum base alloys are used, but because of its present high cost, beryllium cannot be used in large quantities as an alloying constituent in competition with less expensive alloying constituents. We have discovered, however, that by alloying relatively small quantities of beryllium with aluminum there result inexpensive light aluminum base alloys, which, 25 when heat-treated in a particular manner discovered by us, possess materially higher physical properties than previously known similar aluminum-beryllium alloys. This heat treatment is fully described in our Patent No. 30 1,716,943, identified hereinabove.

Aluminum-beryllium alloys such as herein contemplated may be variously manufactured. For example, an alloy of low beryllium content may be prepared by stirring metallic beryllium, 40 which melts at about 1280° C., in molten aluminum at about 1100° C. until the beryllium is dissolved. The use of small amounts of a flux such as barium chloride facilitates introduction of the beryllium. By using higher temperatures, 45 rich aluminum-beryllium alloys containing 10, 25 or 50 per cent or more of beryllium may be prepared in this way for use in the subsequent preparation of aluminum-beryllium alloys having lower beryllium content, or for use themselves without subsequent alloying.

50 The invention will now be further explained with reference to specific examples with the understanding, however, that the examples are given by way of illustrations and not as limitations of the invention.

In the following table there is given in the first column the beryllium content of a number of aluminum-beryllium alloys, specimens of which were prepared by casting the alloys in iron molds to give chill cast slabs about one-fourth of an inch thick. The Brinell hardness values of these alloys as cast were determined by using a 10 millimeter ball under a load of 500 kilograms, and are given in the second column of the table. The several specimens were then all heated for 24 hours at a temperature of 631° C. and then quenched in water, after which their Brinell hardness values given in the third column of the table were determined in the manner just explained. Thereafter the specimens were all permitted to age naturally for two days at room temperature, and their Brinell hardness values given in the last column of the table were then determined.

| Beryllium percent | Hardness as cast | Hardness quenched | Hardness when aged 2 days at room temperature |
|-------------------|------------------|-------------------|-----------------------------------------------|
| 0.013             | 16.8             | 15.7              | 16.9                                          |
| 0.025             | 17.2             | 17.2              | 24.3                                          |
| 0.075             | 19.4             | 22.7              | 36.8                                          |
| 0.21              | 21.2             | 23.8              | 37.0                                          |
| 0.40              | 22.8             | 24.1              | 39.1                                          |
| 0.75              | 25.9             | 27.3              | 42.9                                          |

This table shows that the Brinell hardness values of the specimen containing .013% beryllium do not vary materially with heat-treatment, the hardness value of the specimen when quenched and aged being substantially the same as when cast. However, the specimen having a beryllium content of .025% when quenched and aged had a Brinell hardness materially higher than as cast or as quenched, and this is likewise true of the several specimens having beryllium contents greater than .025%. From this it appears that aluminum base alloys containing not less than about .025% beryllium are capable of having their hardness and strength substantially increased by heat-treating them.

The invention is applicable not only to chill castings made of aluminum-beryllium alloys, but also to sand castings, as shown by the following example. Samples of sand cast aluminum-beryllium alloys containing .5% beryllium showed in the cast condition an average tensile strength of about 12,000 pounds per square inch and a Brinell hardness of 21. After aging 11 days at room temperature the samples showed no ap-

preciable change in strength or hardness. Other samples of the same alloy after being heated for 30 hours at 632° C. and quenched in water had a tensile strength of 13,000 pounds per square inch and a Brinell hardness of 23. These heat-treated samples were then permitted to age naturally at room temperature for 11 days, when it was found that their average tensile strength was 17,000 pounds per square inch and their 10 Brinell hardness 36.

The samples thus far given have been of cast aluminum-beryllium alloys, but the invention contemplates wrought, rolled or otherwise worked alloys. As illustrative of this, an alloy containing 0.075% beryllium was forged hot to a bar about five-eighths of an inch square, and after annealing was found to have a Brinell hardness of 16.4. The sample was then heated for 20 hours at 631° C., quenched in cold water, and then 20 permitted to age naturally at room temperature. After so aging for 16 hours its Brinell hardness was 31, and at the end of 72 hours it was 34.

We have found very useful and beneficial effects are produced by the addition of beryllium to 25 aluminum base alloys containing silicon, copper, magnesium, magnesium and silicon, magnesium and copper, and magnesium, copper and silicon. Depending upon the particular alloy in question, the effect of the addition of beryllium to these 30 alloys may, for example, be to confer age hardening characteristics where they did not exist before, to increase the age hardening characteristics already inherent in the alloy, and to increase the total hardness of the alloy.

35 As shown by the following example, beryllium confers age-hardening properties upon chill cast aluminum-copper alloys. Such an alloy containing 4% copper and no beryllium after being chill cast showed no appreciable increase in hardness after standing several days at room temperature. However, when .05% of beryllium was added to an aluminum base alloy containing 4% copper and the alloy chill cast, the Brinell hardness increased from 46 immediately after casting 40 to 69 after the sample was aged naturally for five days at room temperature. Similarly, the Brinell hardness of an aluminum alloy containing 3% copper and 0.05% beryllium increased from 48 as cast to 64 after aging eight days at 45 room temperature. After heating samples of the last mentioned aluminum-copper-beryllium alloy for eight hours at 589° C. and quenching in water, it was found that the Brinell hardness as quenched was 58, and after aging two days 50 at room temperature it was found that the hardness had risen to 87. Results of the same order were obtained by varying the beryllium as well as the copper content of other aluminum base 55 alloys containing these constituents.

60 Heat-treated pure aluminum-copper alloys show distinct hardening at room temperature. For example, an aluminum-copper alloy containing 4% copper was heat-treated at 550° C. and quenched. The hardness of the as quenched 65 specimen was 63. After aging twenty-five days at room temperature, the hardness had increased to 79. The addition of beryllium to such an alloy causes an increase in this effect. The addition of 0.05% beryllium to the foregoing alloy caused 70 the hardness to increase from 65 immediately after quenching from 550° C. to 99 after aging twenty-five days at room temperature.

75 It is shown in the following example that the addition of beryllium to aluminum-copper alloys has the further advantage of reducing the lia-

bility of the alloy "burning" during its forging or heat-treatment. The heating curve showing the increase in temperature per unit of time of an aluminum-copper alloy containing 6% copper normally shows an arrest when the alloy reaches a temperature of about 548° C., this being due to the fusion of the aluminum-CuAl<sub>2</sub> eutectic at this temperature. When .81% of beryllium was added to an aluminum-copper alloy containing 6% copper and the resulting alloy 80 heated, it was found that the first arrest in the heating curve was at 564° C. and that forgings of this alloy heat-treated for two and one-half hours at 554° C. showed no signs of "burning". This indicates that the copper and beryllium 85 had probably combined in some way, because otherwise any free CuAl<sub>2</sub> present in the alloy would have melted at or below the aluminum-CuAl<sub>2</sub> eutectic temperature of about 548° C. 90

We have found that in some cases heat treatment periods much shorter than some of those used in the preceding examples produce equally beneficial results. As illustrative of this, samples of a forged aluminum-copper-beryllium alloy containing 6% copper and .81% beryllium 95 were heat-treated for two and one-half hours at 554° C. and quenched in water. As determined by using a 1000 kilogram load, the Brinell hardness of this alloy as quenched was 69, and after aging naturally at room temperature for 100 twenty-four hours it had risen to 98. At the end of forty-eight hours the Brinell hardness was 99, and at the end of twelve days it was 101. The average tensile strength of forged samples of this alloy after aging twelve days was found 105 to be about 52,000 pounds per square inch, and the elongation to be 25% in two inches. 110

As to the effects of beryllium on aluminum base alloys containing additional alloying constituents other than copper, we have found by a number 115 of tests that the addition of silicon to aluminum-beryllium alloys results in an increase of their final hardness after quenching. An aluminum base alloy containing .1% beryllium, .5% magnesium and 1% silicon was found to have a 120 Brinell hardness of 42 as cast and of 54 after aging for one week at room temperatures, the latter being materially higher than that of a similar alloy not containing beryllium. After being heated for eighteen hours at 550° C., 125 quenched in water and aged for one week at room temperature the Brinell hardness of the aluminum - beryllium - magnesium - silicon alloy just described was found to be 74. An alloy of the same composition plus 4% copper showed as 130 cast a Brinell hardness of 70, and after aging at room temperature for one week it showed a Brinell hardness of 84. Samples of this alloy, after being heated for fifty hours at 500° C. and quenched in water, showed as quenched a Brinell 135 hardness of 57, and after aging at room temperature for one week a Brinell hardness of 97.

Beryllium also modifies the physical properties of aluminum base alloys containing magnesium, as we have found by tests made on such an alloy 140 containing 10.0% magnesium to which .025% of beryllium was added. For some purposes, copper may advantageously be added to aluminum base alloys containing magnesium. The approximate range of magnesium content over which 145 the beneficial effect of beryllium additions on the physical properties is manifested lies between 0.1% and 10.0%. Where magnesium and copper are both present, we prefer to use the lower end of the permissible range of magnesium con- 150

tent, as for example, where copper is present in amounts of from 2.5% to 6.0%, the magnesium need not, and preferably should not, exceed about 1.5%. We contemplate the addition of 5 beryllium in amounts of between about 0.025% and 1.0% to alloys containing between about 0.1% to 10.0% of magnesium and containing between about 0.1% and 6.0% of copper, and the results of our tests indicate that the advantages of our 10 invention are realized to an appreciable degree with alloys falling within these limits of composition.

Throughout this specification, and in the appended claims, the expression "aluminum base 15 alloy" is used to describe an alloy in which aluminum is the predominant constituent regardless of whether the alloy is binary, ternary, or of a more complex order.

According to the provisions of the patent 20 states, we have explained the principle and mode

of operation of our invention and have described numerous specific examples of the manner in which it may be practiced. However, we desire to have it understood that, within the scope of the appended claims, the invention may be practiced in alloys having compositions differing from those particularly described.

We claim:

1. An aluminum base alloy containing from about 0.025 per cent to 1.0 per cent beryllium, about 1.0 per cent to 10.0 per cent magnesium, and characterized by high hardness and beneficial age hardening properties. 85

2. An alloy consisting of from about 0.025 per cent to 1.0 per cent beryllium, from about 1.0 90 per cent to 10.0 per cent magnesium, and the rest aluminum. 90

ROBERT S. ARCHER.

WILLIAM L. FINK.

95

25

100

30

105

35

110

40

115

45

120

50

125

55

130

60

135

65

140

70

145

75

150